

W. E. OAKLEY.

VALVE.

APPLICATION FILED JUNE 12, 1914.

1,175,172.

Patented Mar. 14, 1916.



Fig. 1.



Fig. 2.



Fig. 3.

Witnesses.

R. D. Tolman.

Penelope Lumberback.

Inventor  
William E. Oakley.

By Fowler & Kennedy

Attorneys

# UNITED STATES PATENT OFFICE.

WILLIAM E. OAKLEY, OF BAYONNE, NEW JERSEY.

## VALVE.

1,175,172.

Specification of Letters Patent. Patented Mar. 14, 1916.

Application filed June 12, 1914. Serial No. 844,786.

*To all whom it may concern:*

Be it known that I, WILLIAM E. OAKLEY, a citizen of the United States, residing at Bayonne, in the county of Hudson and State 5 of New Jersey, have invented a new and useful Improvement in Valves, of which the following, taken in connection with the accompanying drawings, is a specification.

The present invention relates to valves 10 adapted for use within the cylinders of internal combustion engines, to control the intake of gases thereto, and the exhaust of gases therefrom.

It is an object of the present invention to 15 provide a valve possessing the characteristics of strength and ability to resist high degrees of heat as to render its use in the cylinders of engines of this type free from the attendant difficulties which are common 20 to valves now ordinarily used.

Owing to the high temperatures prevailing 25 in the cylinders of internal combustion engines, it has been the practice heretofore to manufacture such valves from metals or alloys of metals calculated to resist the 30 weakening and distorting effects of heat, and consequently valves made of certain alloys of steel, such as nickel steel and tungsten steel, have largely superseded all others, 35 owing to the superior heat resisting qualities found to be possessed by such alloys. However, even with the use of such alloys, the 40 surface pitting of the valves, due to the gaseous corrosion produced by intense heat, and the deposit thereon of carbon, resulting from 45 imperfect combustion of gases and the burning 50 of lubricants within the cylinder, are still a source of constant annoyance, owing to the imperfect and inefficient seating of 55 the valves when thus affected.

The present invention aims to produce a 60 valve adapted to obviate the above objectionable features, and to this end contemplates the manufacture of such a valve from 65 an alloy not heretofore employed in the manufacture of internal combustion engine valves, but which, it has been discovered, possesses characteristics and properties 70 which render it peculiarly adaptable to such a use. Such an alloy consists of a large percentage of nickel, which metal constitutes 75 the base thereof, a considerable percentage of copper, and a very small percentage of iron, thereby differing radically from 80 the alloys previously employed in the manu-

facture of such valves, in all of which iron 85 constitutes the base.

I have illustrated one embodiment of my 90 invention in the accompanying drawings, in which—

Figure 1 is a vertical cross section through 95 a portion of an internal combustion engine cylinder, showing the application of a valve to the exhaust port thereof. Fig. 2 is a side view of a valve. Fig. 3 is a fragmentary 100 section through the stem of a valve, showing a modified construction.

Like reference characters are used to 105 designate like parts in the different views.

Referring to the drawings, 1 denotes the 110 cylinder of an internal combustion engine, which may be of any well known type of construction, and 2 represents a puppet valve adapted to control either the inlet of gas to, or the exhaust of gas from the cylinder 1, in the manner common to engines of this type. In the present instance, the valve co-operates with a seat 3, to control communication between the interior of the cylinder and an exhaust passage 4. The 115 raising of valve 2 from its seat, by the action of any valve operating mechanism, ordinarily employed in connection with engines of this type, permits the escape of exhaust gases past said seat and into the passage 4. 120 It is to be understood that the construction above described is equally applicable to the inlet passage of the cylinder, the valves for both inlet and exhaust being identical in 125 construction.

The valve 2 comprises a head 5, having a 130 suitably beveled seating surface 6 and a stem 7 integral with said head. The valve is made from an alloy, the constituents of 135 which are approximately as follows:—

|        |                |
|--------|----------------|
| Nickel | About 67%.     |
| Iron   | From 1% to 5%. |
| Copper | Remainder.     |

Such an alloy contains but a trace of carbon; it has been found to possess a coefficient of expansion under the application of heat substantially identical with that of the steels ordinarily used in the manufacture of gas engine puppet valves, and also with 105 that of cast iron of which the cylinders are usually made. This alloy is distinguished further by its ability to resist the destructive action of high temperatures, and its 110 freedom from the gaseous corrosion ordi-

narily produced in other metals by the heating of the same above a red heat. It has been found that the alloy does not scale, as does steel, under high temperatures, but 5 that the oxid forms a thin adherent coating. When heated to the maximum temperatures attainable in the ordinary operation of gas engines, this alloy retains approximately 80% of its elastic limit and tensile strength 10 as compared with approximately 71% retained by the best high grade steel at such temperatures. Furthermore, the virtual freedom of this alloy from any carbon content, as compared to the appreciable carbon 15 content of all steel and irons used heretofore in the production of valves of this type, has the effect of eliminating a very potent agency in the production of a deposit of carbon on the valve, namely, the tendency of 20 the carbon produced by combustion of the gas to unite with any carbon contained in the highly heated valve.

The stem of the valve is suitably recessed, as at 8, to receive a washer or collar 9 to 25 form a bearing for the spring 10 which maintains the valve on its seat. The end of the stem 7 is drilled to receive the spindle of a button 11, which may be made of case hardened and tempered steel, adapted to 30 resist the wear occasioned by its contact with the cam 12, which is employed to raise the valve against the action of the spring 10.

In the form shown in Fig. 2, the drilled 35 hole in the end of the stem 7 is screw threaded and the spindle of the button is

screwed therein. In the form shown in Fig. 3, the spindle of the button is made slightly larger than the hole in the stem, and is shrunk therein, by raising the temperature of the end of the stem to permit insertion of 40 the spindle. In either case the button is removable for replacement when the same becomes worn through continued use.

I claim,

1. A valve for internal combustion engines, made from an alloy comprising a large proportion of nickel, and a small proportion of iron.

2. A valve for internal combustion engines, made from an alloy chiefly consisting of 50 nickel and copper.

3. A valve for internal combustion engines, made from an alloy comprising approximately sixty-seven per cent. of nickel and thirty per cent. of copper.

4. A valve for internal combustion engines, made from an alloy consisting of approximately sixty-seven per cent. of nickel, twenty-eight to thirty-two per cent. of copper, and from one to five per cent. 60 of iron.

5. A valve for internal combustion engines made from an alloy consisting chiefly of nickel, and substantially free from carbon.

WILLIAM E. OAKLEY.

Witnesses:

PENELOPE COMBERBACH,  
NELLIE WHALEN.